

# UNITED STATES PATENT OFFICE.

JULES LEURQUIN, OF UCCLE-STALLE, BRUSSELS, BELGIUM.

REPRODUCING PICTURAL, ARTISTIC, AND GRAPHIC WORKS.

1,304,071.

Specification of Letters Patent.

Patented May 20, 1919.

No Drawing.

Application filed October 28, 1916. Serial No. 128,229.

To all whom it may concern:

Be it known that I, JULES LEURQUIN, a subject of the King of Belgium, and resident of Uccle-Stalle, Brussels, Belgium, 214 Avenue Kersbeek, have invented certain new and useful Improvements in Reproducing Pictural, Artistic, and Graphic Works; and I do hereby declare the following to be a full, clear, and exact description of the invention, such as will enable others skilled in the art to which it appertains to make and use the same.

The present invention relates to a new process for reproducing, by printing with oil-colors, pictural, artistic and graphic works of all kinds and specially those belonging to art, sciences, teaching, social organization, politics, agriculture, industry and trade, more particularly: old or modern pictures and decorations, painted in oil-colors or with any other substances, aquarelles, pastel, charcoal, or other drawings, prints, images, posting-bills, geographical maps, ornamenting or tuition boards for schools, architects' plans, and printed matters of all kinds intended to a great diffusion, upon all products of nature or industry having surfaces adapted to be coated or impregnated with agglutinating materials and, more especially, upon vegetable or animal tissues, skins and leathers, upon fabrics made of flax, hemp, cotton, jute, wool, hairs or feathers, natural or artificial silk; upon blades of metal, wood, paper, ivory and natural or artificial nacre.

The process comprises the method of preparing the surfaces intended to be printed and to be so converted into reproductions of the original models.

This method of preparation comprises the following operations:

The fabrics, cloth, or substance in the form of blades intended to be printed are cleaned; the knots, big threads and other defects of the fabric are eliminated. The surfaces on which the works will be reproduced are then smoothed by means of pumice-stone, with or without addition of water, and even in some cases they are rubbed with emery-stone or sand-paper and in the dry state. They must then be coated with a protective gluing material or sizing coat.

After the preparatory operations, the

surfaces are provided with a first layer of 55 the special coating intended to render them capable of being printed.

This coating is prepared by means of white linseed-oil thickened by heating it with or without litharge, until it has acquired a consistency similar to that of the pear syrup. White colors in powder are mixed with that oil; those colors must be neutral in order to avoid blackening of the surfaces. This mixture of colors with 65 thick oil is diluted, before being applied, by means of naphtha, benzene or another volatile material.

The coating is composed in the following manner:

A.—First mixture comprising:

7 parts of oméa-white, first quality.

1 part of baryta-white.

2 parts of zinc-white, first quality.

2½ parts of whitened linseed-oil.

B.—Second mixture:

5 parts of oméa-white.

5 parts of zinc-white, first quality.

3 parts of whitened linseed-oil.

These mixtures are malaxated.

C.—First coating:

5 parts of the first mixture.

2 parts of thick oil.

1 part of volatile essence.

1/10 part of drier or siccative.

D.—Second coating:

6 parts of the second mixture.

3 parts of thick oil.

2 parts of volatile essence.

1/10 part of drier or siccative.

For the substances used as support which must be covered with two layers, the first layer will be of the first coating (C) and the second layer of the second coating (D); for those substances which must be covered with three layers, two layers will be of the first coating (C) and one layer of the second coating (D); these layers are applied by means of a scraper.

E.—Third coating.

2 parts of the second coating (D)

3 parts of volatile essence.

This last mentioned coating is used for the last layer and it is applied by means of a brush.

The proportions of the materials in the various mixtures and coatings may be varied within certain limits, specially according

to the thickness of the substances to be coated.

A first layer of coating is applied on the fabric, and the latter, which is then technically called coated fabric or coated surface, is afterward dried in daylight and in a current of air in order to facilitate the evaporation of the volatile materials and the drying without necessity of using high temperatures; the daylight whitens the surfaces. After several days drying and whitening, the fabric is carefully cleaned by means of a knife, a grater, pumice-stone, emery, granite or in any other suitable manner.

A second and, eventually, several other layers are then applied each of which is dried and whitened in the manner hereinbefore described.

20 A subsequent layer is then applied, dried and whitened. When dried, the fabric is pumicated or smoothed by means of pumice-stone, sandstone, granite, emery, artificial pumice or any other suitable material. The 25 surface acquires then an appearance similar to that of paper and very suitable for printing. According to the quality of the product to be made, the application of a layer followed by a pumicing operation may 30 be repeated several times. It is possible to obtain in this way a final surface possessing a receptivity quite similar to that of paper, as far as printing is concerned, but having besides the strength, suppleness and flexibility of the fabric, a great suppleness remaining in the fabric owing to the use of thick or agglutinated oil which is the only agglomerating material which remains in the dried coating.

40 In some cases, it is advantageous to give to the surface intended for printing a dull but whiter appearance, which is performed by applying an additional layer, the purpose of which is also to render the impression 45 more adherent. This last layer has the same composition as the coating previously used, but with a far greater proportion of volatile

liquid (naphtha, benzene), so as to have a product more diluted. This last layer is not pumicated at all.

50

When the substance prepared is intended to be used for the reproduction of certain artistic works, a quantity of the material known as amber-oil or "huile d'ambre" may be mixed with the color of the last layer, in 55 order to vary the tint of the colors. Said addition must be made in a proportion determined according to the effect desired.

When artistic works are reproduced, it is advantageous to make an impression with 60 colors without relief, followed by an application of colors in relief; this last mentioned application may be performed either by a printing process or by hand.

By these means, it is possible to reproduce 65 integrally the original works with all their characteristics: impastations, tints, shadows, clear-obscuré, light, perspective, without any exception, including the distinctive signs denoting the origin thereof.

70

What I claim is:

1. A process for reproducing pictorial, artistic and graphic works, consisting in preparing a mixture of colors, thickened linseed-oil and a volatile liquid, applying 75 said mixture in several layers on a supporting substance, drying and pumicating each layer and printing on the coating formed by said layers.

2. A process for reproducing pictorial 80 artistic and graphic works, consisting in coating a supporting substance with a mixture of colors, thickened linseed oil and a volatile liquid and applying to said substance a subsequent layer containing a mixture of colors, thickened linseed oil, a volatile liquid and amber oil, and printing on the coating formed by said layers.

In testimony whereof I affix my signature in presence of two witnesses.

JULES LEURQUIN.

Witnesses:

CHARLES MERCHIS,

CHARLES ROY NASWITH.

Copies of this patent may be obtained for five cents each, by addressing the "Commissioner of Patents, Washington, D. C."